# EUROPEAN PATENT SPECIFICATION

(11) **EP 3 504 717 B1**
(45) Date of publication and mention of the grant of the patent: **27.05.2020**
(21) Application number: 17772163.6
(22) Date of filing: 07.09.2017
(51) Int. Cl.: G21G 4/06

(54) **LOW DENSITY POROUS IRIDIUM**
PORÖSES IRIDIUM MIT NIEDRIGER DICHTE
IRIDIUM POREUX À FAIBLE DENSITÉ

(30) Priority: 19.05.2017 WO PCT/US2017/033508
(43) Date of publication of application: 03.07.2019
(73) Proprietor: QSA Global Inc., Burlington, MA 01803 (US)
(72) Inventor: SHILTON, Mark, G., Chelmsford, MA 01824 (US); VOSE, Mark, W., Windham, NH 03087 (US)
(74) Representative: Trinks, Ole
(86) International application number: PCT/US2017/050425
(87) International publication number: WO 2018/084929

(56) References cited:
- WO-A1-2015/175326
- US-B1- 7 118 729

## Description

### BACKGROUND OF THE DISCLOSURE

This application claims priority from PCT/US2017/033508, entitled "Low Density Spherical Iridium", filed on May 19, 2017.

### Field of the Disclosure

The disclosure pertains to a gamma radiation source, typically containing microbeads of iridium, or low-density alloys or compounds or composites of iridium and porous variants of these.

### Description of the Prior Art

The prior art of radiation sources of various types for medical, industrial and other processes is well-developed. However, further improvements are sought, particularly with respect to manufacturing economies and product performance.

A prior art method for producing a gamma ray source is disclosed in PCT/NL2004/000401 (also published as WO 2004109716 A2) to Bakker Klass. This method includes the steps of neutron irradiation of disks of iridium or cobalt, and stacking the disks to form a cylinder. Similarly, the prior art includes PCT/US2015/029806 (also published as WO 2015175326 A1) entitled "Device and Method for Enhanced Iridium Gamma Radiation Sources"; German Patent Document DE 19824689 C1 with a translated title "Iridium-Containing Molding useful as a Gamma Radiation Source e.g., For Weld Seam Radiography and Cancer Treatment"; and PCT/US2015/029806 entitled "Device and Method for Enhanced Iridium Gamma Radiation Sources."

Further prior art relating to the manufacture of metallic spheres includes U.S. Patent No. 2,394,727entitled "Method for Making Small Metallic Spheres", issued on February 12, 1946 to Taylor, and information found at:
http://www.orau.org/ptp/collection/sources/3mdisk.htm; and
http://www.nrc.gov/docs/ML0415/ML041550720.pdf.

Methods of manufacturing porous iridium can be found in "The Metallurgical Integrity of the Frit Vent Assembly Diffusion Bond," by G.B. Ulrich, June 1994, Document Y/DV-1321, Oak Ridge Y-12 Plant, Martin Mariette Energy Systems, Inc.

### OBJECTS AND SUMMARY OF THE DISCLOSURE

It is therefore an object of the present disclosure to provide improvements in the radioactive sources used in medical and industrial applications. Embodiments of the disclosure may achieve many of the following objectives with respect to the prior art - reduced fabrication costs, reduced focal dimensions (particularly with respect to cylindrical geometry natural iridium disk sources), increased activation yield, increased output (more output Ci/mg due to reduced density), a softer emission spectrum due to low reduced density (i.e., more predominant lower energy emissions) and a near spherical, or quasi-spherical geometry (resulting in improved image quality), but typically including flat sides around its circumference in order to avoid infinitely sharp tangential lid components. Additionally, handling of radioactive powders can be reduced or eliminated in embodiments of this disclosure.

It is envisioned that embodiments of the present disclosure could increase lridium-192 output efficiency, perhaps in the range of 11-17 percent, particularly if sources could be made using 50 to 65 percent dense iridium with spherical or quasi-spherical geometry. This could further result in a reduction of 11 to 17 percent in Iridium-192 source content and annual consumption. Additionally, the softer output spectrum combined with near-spherical focal geometry could result in image quality approaching that of cylindrical enriched Iridium-192 sources. It is further envisioned that this could potentially lead to an increased activation yield of 7-11 percent leading to an overall 18-28 percent efficiency gain.

Optionally, flat-faced disks of low-density porous iridium or a compound, alloy, composite or porous variant thereof can be activated to produce disks containing Ir-192. After activation, disks can be stacked to form spherical or quasi-spherical focal geometries.

Disks of low-density porous iridium or a compound, alloy, composite or porous variant thereof having curved, domed or otherwise shaped faces can be made so that they are thicker in the middle than at the circumference. Some practical examples are shown in figure 4. These can be activated to produce disks containing Ir-192. After activation, such disks can be stacked and then compressed, compacted or deformed to produce spherical or quasi-spherical focal geometries. Disks that are shaped in this way may be more easily converted into spherical or quasi-spherical focal geometry by compression, compaction or deformation as shown in figure 5, leading to manufacturing advantages.

The use of spherical or quasi-spherical low-density Iridium-192 or a compound, alloy, composite or porous variant thereof could achieve similar yield and output efficiency gains that have been achieved with annular iridium, but without image quality or focal dimension disadvantages of annuli stacked in a cylindrical configuration.

Alternately spherical or quasi-spherical low density Iridium-192 or a compound, alloy, composite or porous variant thereof could also be made using random-packed or partially random packed microgranules in a spherical or quasi-spherical source cavity. Porous microgranules may be compressed, compacted or deformed to produce spherical or quasi-spherical focal geometries.

It should be noted that the pore size within porous iridium or a compound, alloy, composite or porous variant thereof may vary and be in the range from sub-micrometer dimensions (sometimes referred to as microporosity) to approximately sub-millimeter dimensions (sometimes referred to as porosity).

Porous iridium or a compound, alloy, composite or porous variant thereof may be made by several different methods. One method is to heat microspheres or micro-granules at a temperature, typically above 1000°C, but more typically above 1300°C for a time period long enough to initiate durable bonding and fusion at their points of contact.

Microporous iridium or a compound, alloy, composite or porous variant thereof may also be made by partially sintering finely divided powder at a temperature, typically above 1000°C, but more typically above 1300°C for a time period long enough to initiate durable interparticle bonding and fusion at their points of contact, but not long enough to complete the densification process. Such a microporous product will have a density less than one hundred percent of the theoretical density of iridium, due to the voids, pockets or channels formed within the iridium or iridium alloy, compound or composite.

Isotopically enriched iridium-191 powder can be used as a raw material for making low density porous iridium or a compound, alloy, composite or porous variant thereof. This form of iridium can be made by gas-centrifuge isotopic enrichment of gaseous natural isotopic abundance iridium hexafluoride or iridium tetrafluoride by reducing the enriched process gasses to produce a highly amorphous form of elemental enriched iridium-191, often referred to as iridium-black. The iridium produced by such processes lacks crystallinity, has a very small average particle size (typically sub-nanometer), has a very high internal surface area and is porous.

It has been found that such amorphous (or substantially amorphous) iridium powder can be cold-compressed to form compacts having 30-50% of the theoretical density of iridium. These can be partially densified, bonded and fused by sintering at an unexpectedly low temperature, well below the temperature that is common for crystalline materials. The high surface energy due to high internal surface area and high amorphous lattice energy may drive densification, crystallization, grain growth and interparticle fusion at lower than expected temperatures.

It has been found that partial densification of substantially amorphous pure iridium powder, such as the material produced by gas a centrifuge enrichment process, can be achieved at temperatures as low as 1300°C. Moreover, the addition of certain sintering additives that are non-activating, low-activating or compatibly-activating (i.e. producing minimal interfering gamma ray emissions), and having lower melting point than iridium can form alloys, intermetallic compounds or combinations thereof with iridium. Such additives include, but are not limited to aluminum, vanadium, boron-11, silicon, phosphorous, sulfur, carbon, beryllium, titanium, nickel, tungsten or alloys and intermetallic compounds thereof, which further lower the sintering temperature and may enhance the partial densification process and/or improve ductility to achieve superior bonding with improved mechanical properties at a lower temperature and time.

Finely divided amorphous or substantially amorphous Iridium powder having natural isotopic composition can also be similarly partially densified and bonded.

Partially densified, bonded, porous, low-density, iridium components can be made in the form of disks, cylinders, wires, granules or microspheres. These can be stacked or otherwise assembled together and then compressed, compacted or mechanically deformed to produce a spherical or quasi-spherical focal geometry, which is both optimum for radiography source manufacturing and for radiographic image quality.

The focal dimension of the spherical or quasi-spherical low density Iridium-192 would typically be no larger than the diagonal of a conventional stacked-disk 100% dense cylindrical source geometry.

The resulting sources would emit lower energy gamma rays leading to improved image contrast and resolution.

### BRIEF DESCRIPTION OF THE DRAWINGS

Further objects and advantages of the disclosure will become apparent from the following description and from the accompanying drawings, wherein:
Figure 1 is a flowchart of a typical manufacturing process of the present disclosure, with variations being envisioned.
Figure 2 illustrates calculated gamma energy spectral abundances as a function of iridium density in accordance with an embodiment of the present disclosure.
Figure 3 illustrates the volume ratios of cylindrical stacks vs. spheres having the same focal dimension and the typical increase in emissivity and irradiation yield achieved with an embodiment of the present disclosure.
Figure 4A is a side plan view of disk design options of the present disclosure.
Figure 4B is a side plan view of a prior art disk design.
Figure 5A is a side plan view of a disk stack prior to compression, compaction or deformation to produce a sphere or quasi-sphere.
Figure 5B is a side plan view of a preferred embodiment of a disk stack after compression, compaction or deformation thereby producing a sphere or quasi-sphere.
Figure 6 illustrates disk stacking without compression, compaction or deformation to spherical / quasi-spherical geometry using hemi-discus-shaped end pieces.
Figure 7 illustrates a cross-sectional view of a disk comprising bonded microspheres and bonding additives.
Figures 8A and 8B illustrate the shiltoid and vosoid shapes, respectively, as defined by the applicants.
Figure 9 is a plan view of an embodiment of a disk of the present disclosure.
Figure 10 is a cross-sectional view along plane 10-10 of Figure 9.

### DETAILED DESCRIPTION OF THE PREFERRED EMBODIMENTS

Referring now to the drawings in detail, one sees that Figure 1 is a global schematic of a typical process 100 underlying the present disclosure. Natural iridium is provided at block 102, 102' or 102". Natural iridium at block 102 is provided directly to the block of making disks or microgranules 110. Natural iridium at block 102' is alloyed or provided with sintering additives at block 108 and then provided to the block of making disks or microgranules 110. Natural iridium at block 102" is provided to the gas centrifuge enrichment block 104, the enriched iridium block 106, and optionally, alloyed or provided with sintering additives at block 108, before being provided to the block of making disks or microgranules 110 The microgranules or microbeads typically have a diameter of 0.25 - 0.60 mm., preferably 0.40 mm. in many embodiments.

Iridium, in a disk or microgranule form, from block 110, regardless of the origin (102, 102' or 102") is optionally provided to block 112 for partial densification, such as by sintering or some other technique. The iridium is subsequently optionally supplied to the laser seal surface block 114, and then the activate and measure blocks 116, 118, respectively. As shown in the upper branch of the diagram, the iridium from the measure block 118 may be loaded into a capsule at block 120, optionally compressed, compacted or deformed in the capsule at block 122 and then the source is welded at block 128. Alternately, as shown in the lower branch of the diagram, the iridium from measure block 118 may be first stacked and compressed, compacted or deformed at block 124 prior to being loaded into a capsule at block 126 (similar to block 120) and then the source is welded at block 128.

Referring to Figure 2, one sees a typical gamma energy spectrum showing calculated spectral abundances as a function of iridium density for lower density iridium in accordance with the type of processes summarized in Figure 1.

Similarly, referring to Figure 3, one sees a typical increase in emissivity and radiation yield compared with prior art 100 percent dense iridium and proportionally higher emission at lower energies. It is noted for example, that a fifty-three percent dense sphere of a given diameter "d" (such as, but not limited to, 3.82 millimeters) has eighty-nine percent more volume than a 100 percent dense right cylinder, with a 3.82 mm. diagonal "d". Such a right cylinder has a height and diameter both equal to 2.7 mm. (3.82 mm. divided by the square-root of 2.0). These dimensions are quite typical of the active-dimensions of standard cylindrical 100 Ci Iridium-192 sources containing natural Iridium-192. However, the referenced sphere or quasi-sphere has the same focal dimension and estimated eleven to seventeen percent higher output than the referenced right cylinder (note that the relative increase in output depends on the direction the emission is measured in: axial, radial, 4π or other). It is therefore expected that spherical or quasi-spherical low density iridium-192 increases source output efficiency in the approximate range 11 - 17 percent. With an expected reactor yield increase in the range of 7 -11 percent, it is expected that the combined reactor yield plus output efficiency increase will be on the order of 18 - 28 percent.

Figure 4A illustrates examples of compressible, compactable or deformable disk profiles which may be implemented in accordance with the type of processes summarized in Figure 1. As opposed to the illustrated prior art design of Figure 4B wherein a conventional flat disk profile is produced by a shallow cylindrical shape, the disk 10 of Figure 4A is approximated by the rotation of an ellipse about its minor axis (also see Figures 9 and 10 for a somewhat similar shape). Alternative disk profiles are chosen from one of the various illustrated profiles 11 (a flat central cross-sectional area with sharp pointed circumferential edges), 12 (a flat central cross-sectional area with dull pointed circumferential edges), 13 (a flat narrow central cross-sectional area with dull pointed circumferential edges), 14 (a flat narrow central cross-sectional area with gently rounded circumferential edges), 15 (a discus or ellipsoid shape with somewhat rounded circumferential edges), 16 (a thinner discus or ellipsoid shape with somewhat rounded circumferential edges) and 17 (a discus or ellipsoid shape with somewhat rounded circumferential edges and a center portion 18 which is translated upwardly in the orientation of Figure 4A to provide a stack alignment characteristic, so that a plurality of stacked disks 17 can sequentially nest with each other). These disks are typically 0.1 to 0.7 mm. thick, and typically do not exceed 0.75 mm. in thickness.

Figure 5A illustrates a stack of the disks 10 (or alternately, any of 11 through 17) prepared for compression, compaction or deformation (see blocks 122 and 124 of Figure 1)to form the spherical or quasi-spherical irradiation source 90 of Figure 5B.

An alternative embodiment of an irradiation source 90 as shown in Figure 6 contains Iridium-191 in the form of a metal, alloy, compound, composite or porous variant of the above optimum iridium density range of the active insert (chosen from 30-85 percent, 40-70 percent or 50-65 percent) in which hemi-discus-shaped, hemi-ellipsoid or chamfered endpieces 22, 24 are placed at each end of a stack of flat disks 26. The disks 26 may optimally be approximately 0.25 mm. thick or up to a maximum of about 0.5 mm. thick to maximize activation efficiency and minimize neutron self-shielding during activation. The curved end pieces 22, 24 may optimally be approximately be 0.5 mm. thick in the center or up to a maximum of about 0.75 mm. thick in the center to maximize activation efficiency and minimize neutron self-shielding during activation. This forms a cylinder with curved (or chamfered) ends (similar to a domed vosoid or shiltoid shape).

A shiltoid, as coined by the applicants and as illustrated in Figure 8A, is formed by rotating an octagon about its vertical axis. Likewise, a vosoid, as coined by the applicants and as illustrated in Figure 8B, is formed by inscribing an octagon within a circle, retaining the alternating octagonal walls which form the top, bottom and vertical sides while retaining the circular portions for the remaining portions, and then rotating the resulting shape about its vertical axis. Although the geometry in Figure 6 is less spherical in shape than the preferred shapes, this may have other advantages. It could enable conventional disk irradiations to be carried out using conventional irradiation target geometry.

A further alternative includes the use of porous iridium, possibly including a non-activating, low-activating or compatibly-activating sintering additive or binder such as, but not limited to aluminum, vanadium, boron-11, silicon, phosphorous, sulfur, carbon, beryllium, titanium, nickel, tungsten or any of their alloys such as DOP26 alloy and intermetallic compounds thereof. Additionally, some platinum-192 and osmium-192 may be created *in situ* as a β∼' decay product of Iridium-192. Depending upon the specific elemental proportions or physical states of the composite, compound or alloy, varying degrees of ductility and bonding may be achieved. Lower ductility configurations may be brittle resulting in fracture in response to stress. Higher ductility configurations may allow for the composite, compound or alloy to be compressed, compacted or deformed into the desired shape, such as, but not limited to a sphere or quasi-sphere.

Additionally, under some circumstances, milling with sufficient physical impact may allow the iridium and such additives as aluminum or vanadium to bond or alloy-bond (that is, an alloy is formed at the immediate areas of intersection between the iridium particles and the additive particles). Cold pressing iridium with an aluminum or vanadium additive may produce a resulting product with an iridium density less than 100 percent (due to the presence of the additive and/or porosity).

Moreover, liquid sintering may be performed using a liquid additive, such as, but not limited to, aluminum heated above its melting point, which may be melted *in situ* or poured into a volume of iridium microspheres with a resulting product with an iridium density less than 100 percent (due to the presence of the additive). The liquid additive hardens at a reduced temperature and maintains the iridium microspheres in place. In some embodiments, the microspheres or microgranules may be provided in a single layer bonded with aluminum or vanadium or other compatible low-density bonding metal to form a disk 18 of low-density bonded microspheres or microgranules 40 (see Figure 7), which can be activated using conventional disk irradiation targets, stacked after activation and then compressed, compacted or otherwise deformed to form a spherical or quasi-spherical source insert.

Further possibilities include pressing of iridium in a nanoparticle form (sometimes referred to as "iridium black") which results in an amorphous (non-crystalline) product and an iridium density in the range 30-50%, but more typically about 35 percent, as compared to conventional solid iridium. Similarly, iridium and aluminum, both in nanoparticle form, may be mixed and heated to effect bonding between the particles, and then pressed into a disk.

A domed (discus-shaped) disk for the iridium alloys, compounds or other composites, including porous iridium, can facilitate easier compression, compaction or deformation to quasi-spheres within the active insert as in Figures 4A, 5A and 5B.

In instances when partially sintered or pressed porous low density iridium was excessively friable to be handled without risking breakage or erosion of the surfaces, the disks could be sealed together using soft foil metals (such as, but not limited to, aluminum, titanium or vanadium alloys or other typically non-activating or low-activating alloys). Other options may include laser-melting, sintering or bonding of the surfaces of the disks, similar to the process of laser engraving a solid circle, which may seal and strengthen the surface of the disk. These domed (discus-shaped) disks may be subsequently compressed, compacted or deformed into spherical or quasi-spherical shapes for use in an active insert as shown in Figures 5A and 5B.

Further embodiments of reduced density iridium may be achieved by three-dimensional printing techniques using a reservoir or powder bed of iridium, iridium alloy, composite particles and/or a binder. Such a process may further include subsequent incineration of the binder..

Thus the several aforementioned objects and advantages are most effectively attained. Although preferred embodiments of the invention have been disclosed and described in detail herein, it should be understood that this invention is in no sense limited thereby.

## Claims

1. A radiation source (90) including iridium,
wherein at least a portion of the iridium is porous or microporous iridium, and wherein the density of the active insert containing the iridium is in a range of 30 to 85 percent of the density of 100% dense pure iridium, **characterized in that**
the iridium is in the form of disks (10, 11, 12, 13, 14, 15, 16, 17) having flat, curved or shaped faces that are thicker in the middle than at the circumference, which are stacked, compressed or otherwise formed into a sphere or quasi-sphere, or in the form of microbeads or microgranules (40).

2. The radiation source (90) of Claim 1,
wherein the iridium is in a range of 40 to 70 percent of the density of 100% dense pure iridium, or
wherein the iridium is in a range of 50 to 65 percent of the density of 100% dense pure iridium.

3. The radiation source (90) of Claim 1 or 2,
wherein the pores within the porous or microporous iridium contain a low-density metal, alloy, compound or composite of a non-activating, low activating or compatibly activating additive.

4. The radiation source (90) of one of the preceding claims,
wherein the iridium is in the form of a metal, alloy, compound or composite, prior to neutron irradiation.

5. The radiation source (90) of one of the preceding claims,
wherein the iridium is Iridium-192 contained within a metal, alloy, compound, or composite and formed into a sphere or quasi-sphere.

6. The radiation source (90) of Claim 1,
wherein the iridium disks (10, 11, 12, 13, 14, 15, 16, 17) are between 0.1-0.7mm thick.

7. The radiation source (90) of Claim 5 or 6,
wherein the Iridium-192 is contained within a metal, alloy, compound, or composite material and formed or shaped into a sphere or quasi-sphere by a method of physical compression, compaction or deformation.

8. The radiation source (90) of Claim 1,
wherein the iridium metal, alloy, compound, or composite is in the form of approximately 0,4 mm diameter microbeads or microgranules (40) containing porous iridium-191, prior to neutron irradiation.

9. The radiation source (90) of Claim 1,
wherein the iridium metal, alloy, compound, or composite is in the form of microbeads or microgranules (40) with a diameter of 0.25 - 0.60 mm, containing porous Iridium-191, prior to neutron irradiation.

10. The radiation source (90) of Claim 8 or 9,
wherein the microbeads or microgranules (40) of iridium-191 metal, alloy, compound, or composite are in a random-packed or partly random configuration.

11. The radiation source (90) of Claim 1,
wherein the iridium contains Iridium-191 in the form of a metal, alloy, compound or composite, which is formed into a disk (10, 11, 12, 13, 14, 15, 16, 17), hemi-ellipsoid or other thin flat shape less than 0,75 mm thick, prior to neutron irradiation.

12. The radiation source (90) of one of the preceding claims,
further including a spherical or quasi-spherical source cavity in which the iridium is contained.

13. The radiation source (90) of one of the preceding claims,
wherein the pores within the porous or microporous iridium contain a low-density metal, alloy, compound or composite of a non-activating, low activating or compatibly activating additive, which aids sintering, compaction or deformation, wherein the additive or additives are selected from the group consisting of aluminum, vanadium, boron-11, silicon, phosphorous, sulfur, carbon, beryllium, titanium, nickel, tungsten or alloys and intermetallic compounds thereof.

14. The radiation source (90) of Claim 1,
wherein the iridium is in the form of a metal, alloy, compound or composite, prior to neutron irradiation wherein the additive or additives are selected from the group consisting of aluminum, vanadium, boron-11, silicon, phosphorous, sulfur, carbon, beryllium, titanium, nickel, tungsten or alloys and intermetallic compounds thereof.

## Patentansprüche

1. Strahlungsquelle (90), die Iridium einschließt, wobei mindestens ein Anteil des Iridiums poröses oder mikroporöses Iridium ist, und wobei die Dichte des aktiven Einsatzes, welcher das Iridium enthält, in einem Bereich von 30 bis 85 Prozent der Dichte von 100 % dichtem reinem Iridium liegt, **dadurch gekennzeichnet, dass**
das Iridium in Form von Scheiben (10, 11, 12, 13, 14, 15, 16, 17) mit flachen, gekrümmten oder geformten Flächen vorliegt, die in der Mitte dicker als am Umfang sind, die gestapelt, komprimiert oder anderweitig zu einer Sphäre oder Quasisphäre gebildet worden sind oder in Form von Mikroperlen oder Mikrogranulat (40) vorliegen.

2. Strahlungsquelle (90) nach Anspruch 1,
wobei das Iridium in einem Bereich von 40 bis 70 Prozent der Dichte von 100 % dichtem reinem Iridium vorliegt, oder
wobei das Iridium in einem Bereich von 50 bis 65 Prozent der Dichte von 100 % dichtem reinem Iridium vorliegt.

3. Strahlungsquelle (90) nach Anspruch 1 oder 2, wobei die Poren innerhalb des porösen oder mikroporösen Iridiums ein Metall, eine Legierung, eine Verbindung oder einen Verbund mit niedrige Dichte aus nicht-aktivierendem, gering aktivierendem oder kompatibel aktivierendem Additiv enthalten.

4. Strahlungsquelle (90) nach einem der vorhergehenden Ansprüche, wobei das Iridium vor der Neutronenbestrahlung in Form eines Metalls, einer Legierung, einer Verbindung oder eines Verbunds vorliegt.

5. Strahlungsquelle (90) nach einem der vorhergehenden Ansprüche, wobei das Iridium Iridium-192 ist, das in einem Metall, einer Legierung, einer Verbindung oder einem Verbund enthalten ist und zu einer Sphäre oder Quasisphäre gebildet worden ist.

6. Strahlungsquelle (90) nach Anspruch 1,
wobei die Iridiumscheiben (10, 11, 12, 13, 14, 15, 16, 17) zwischen 0,1 und 0,7 mm dick sind.

7. Strahlungsquelle (90) nach Anspruch 5 oder 6, wobei das Iridium-192 in einem Metall-, Legierungs-, Verbindungs- oder Verbundmaterial enthalten ist und nach einem Verfahren der physikalischen Kompression, Verdichtung oder Verformung zu einer Sphäre oder Quasisphäre gebildet oder geformt worden ist.

8. Strahlungsquelle (90) nach Anspruch 1,
wobei das Iridiummetall, die Iridiumlegierung, die Iridiumverbindung oder der Iridiumverbund vor der Neutronenbestrahlung in Form von Mikroperlen oder Mikrogranulat (40) mit ungefähr 0,4 mm Durchmesser vorliegt, die poröses Iridium-191 enthalten.

9. Strahlungsquelle (90) nach Anspruch 1,
wobei das Iridiummetall, die Iridiumlegierung, die Iridiumverbindung oder der Iridiumverbund vor der Neutronenbestrahlung in Form von Mikroperlen oder Mikrogranulat (40) mit einem Durchmesser von 0,25 bis 0,60 mm vorliegt, die poröses Iridium-191 enthalten.

10. Strahlungsquelle (90) nach Anspruch 8 oder 9,
wobei die Mikroperlen oder das Mikrogranulat (40) aus Iridium-191-Metall, -Legierung, -Verbindung oder -Verbund in einer statistisch gepackten oder teilweise statistischen Konfiguration vorliegen.

11. Strahlungsquelle (90) nach Anspruch 1,
wobei das Iridium vor der Neutronenbestrahlung Iridium-191 in Form eines Metalls, einer Legierung, einer Verbindung oder eines Verbunds enthält, gebildet zu einer Scheibe (10, 11, 12, 13, 14, 15, 16, 17), einem Halbellipsoid oder einer sonstigen dünnen flachen Form mit weniger als 0,75 mm Dicke.

12. Strahlungsquelle (90) nach einem der vorhergehenden Ansprüche,
des Weiteren einschließend einen sphärischen oder quasisphärischen Quellhohlraum, in dem das Iridium enthalten ist.

13. Strahlungsquelle (90) nach einem der vorhergehenden Ansprüche, wobei die Poren innerhalb des porösen oder mikroporösen Iridiums ein Metall, eine Legierung, eine Verbindung oder einen Verbund mit niedriger Dichte aus einem nicht-aktivierenden, gering aktivierenden oder kompatibel aktivierenden Additiv enthalten, welches Sintern, Verdichtung oder Verformung unterstützt, wobei das Additiv oder die Additive ausgewählt ist/sind aus der Gruppe bestehend aus Aluminium, Vanadium, Bor-11, Silicium, Phosphor, Schwefel, Kohlenstoff, Beryllium, Titan, Nickel, Wolfram oder Legierungen und Intermetallverbindungen davon.

14. Strahlungsquelle (90) nach Anspruch 1,
wobei das Iridium vor der Neutronenbestrahlung in Form eines Metalls, einer Legierung, einer Verbindung oder eines Verbunds vorliegt, wobei das Additiv oder die Additive ausgewählt ist/sind aus der Gruppe bestehend aus Aluminium, Vanadium, Bor-11, Silicium, Phosphor, Schwefel, Kohlenstoff, Beryllium, Titan, Nickel, Wolfram oder Legierungen und Intermetallverbindungen davon.

## Revendications

1. Source de rayonnement (90) contenant de l'iridium,
dans laquelle au moins une partie de l'iridium est de l'iridium poreux ou microporeux, et dans laquelle la densité de l'insert actif contenant l'iridium est de 30 à 85 % de la densité de l'iridium pur à une densité de 100 %, **caractérisée en ce que**
l'iridium est sous forme de disques (10, 11, 12, 13, 14, 15, 16, 17) ayant des faces plates, courbes ou formées, qui sont plus épais au milieu qu'autour de la circonférence, qui sont superposés, comprimés ou autrement formés en une sphère ou quasi-sphère, ou sous forme de microbilles ou de microgranules (40).

2. Source de rayonnement (90) selon la revendication 1,
dans laquelle l'iridium est présent à un niveau de 40 à 70 % de la densité de l'iridium pur à une densité de 100 %, ou
dans laquelle l'iridium est présent à un niveau de 50 à 65 % de la densité de l'iridium pur à une densité de 100 %.

3. Source de rayonnement (90) selon la revendication 1 ou 2,
dans laquelle les pores dans l'iridium poreux ou microporeux contiennent un métal, un alliage, un composé ou un composite de faible densité d'un additif non activant, peu activant ou activant de façon compatible.

4. Source de rayonnement (90) selon l'une des revendications précédentes,
dans laquelle l'iridium est sous la forme d'un métal, d'un alliage, d'un composé ou d'un composite, avant l'irradiation neutronique.

5. Source de rayonnement (90) selon l'une des revendications précédentes,
dans laquelle l'iridium est de l'iridium-192 présent à l'intérieur d'un métal, d'un alliage, d'un composé ou d'un composite, et formé en une sphère ou quasi-sphère.

6. Source de rayonnement (90) selon la revendication 1,
dans laquelle les disques d'iridium (10, 11, 12, 13, 14, 15, 16, 17) ont une épaisseur de 0,1 à 0,7 mm.

7. Source de rayonnement (90) selon la revendication 5 ou 6,
dans laquelle l'iridium-192 est présent à l'intérieur d'un métal, d'un alliage, d'un composé ou d'un composite, et formé ou mis en forme pour produire une sphère ou quasi-sphère par un procédé de compression physique, de compactage ou de déformation.

8. Source de rayonnement (90) selon la revendication 1,
dans laquelle le métal, l'alliage, le composé ou le composite d'iridium est sous la forme de microbilles ou de microgranules d'environ 0,4 mm de diamètre (40) contenant de l'iridium-191 poreux, avant l'irradiation neutronique.

9. Source de rayonnement (90) selon la revendication 1,
dans laquelle le métal, l'alliage, le composé ou le composite d'iridium est sous la forme de microbilles ou de microgranules (40) de 0,25 à 0,60 mm de diamètre, contenant de l'iridium-191 poreux, avant l'irradiation neutronique.

10. Source de rayonnement (90) selon la revendication 8 ou 9,
dans laquelle les microbilles ou les microgranules (40) de métal, d'alliage, de composé ou de composite d'iridium-191 sont présents dans une configuration de remplissage aléatoire ou partiellement aléatoire.

11. Source de rayonnement (90) selon la revendication 1,
dans laquelle l'iridium contient de l'iridium-191 sous la forme d'un métal, d'un alliage, d'un composé ou d'un composite, qui est formé en un disque (10, 11, 12, 13, 14, 15, 16, 17), un hémi-ellipsoïde ou une autre forme mince et plate de moins de 0,75 mm d'épaisseur, avant l'irradiation neutronique.

12. Source de rayonnement (90) selon l'une des revendications précédentes,
comprenant en outre une cavité de source sphérique ou quasi-sphérique dans laquelle est contenu l'iridium.

13. Source de rayonnement (90) selon l'une des revendications précédentes,
dans laquelle les pores dans l'iridium poreux ou microporeux contiennent un métal, un alliage, un composé ou un composite de faible densité d'un additif non activant, peu activant ou activant de façon compatible, qui facilite le frittage, le compactage ou la déformation, et dans laquelle l'additif ou les additifs sont sélectionnés dans le groupe constitué de l'aluminium, du vanadium, du bore-11, du silicium, du phosphore, du soufre, du carbone, du béryllium, du titane, du nickel, du tungstène ou d'alliages et de composés intermétalliques de ceux-ci.

14. Source de rayonnement (90) selon la revendication 1,
dans laquelle l'iridium est sous la forme d'un métal, d'un alliage, d'un composé ou d'un composite, avant l'irradiation neutronique, et dans laquelle l'additif ou les additifs sont sélectionnés dans le groupe constitué de l'aluminium, du vanadium, du bore-11, du silicium, du phosphore, du soufre, du carbone, du béryllium, du titane, du nickel, du tungstène ou d'alliages et de composés intermétalliques de ceux-ci.
